# EUROPEAN PATENT SPECIFICATION

(11) **EP 1 647 380 B1**
(45) Date of publication and mention of the grant of the patent: **09.01.2008**
(21) Application number: 05256230.3
(22) Date of filing: 05.10.2005
(51) Int. Cl.: B27N 3/00, D04H 1/54

(54) **Method for manufacturing molded fiber articles**
Verfahren zur Herstellung von Faserformkörpern
Procédé pour produire des objets en fibre moulée

(30) Priority: 12.10.2004 JP 2004297649; 16.03.2005 JP 2005075259
(43) Date of publication of application: 19.04.2006
(73) Proprietor: Toyota Boshoku Kabushiki Kaisha, Kariya-shi, Aichi-ken (JP); Toyota Shatai Kabushiki Kaisha, Kariya-shi, Aichi-ken (JP)
(72) Inventor: Hashiba, Masanori c/o Toyota Boshoku Kabushiki K., Kariya-shi Aichi-ken (JP); Kawajiri, Hideki c/o Toyota Boshoku Kabushiki K., Kariya-shi Aichi-ken (JP)
(74) Representative: Pratt, David Martin

(56) References cited:
- EP-A- 0 237 665
- EP-A- 1 400 328
- GB-A- 1 453 503
- US-A- 4 292 105
- US-A1- 2004 180 990
- PATENT ABSTRACTS OF JAPAN vol. 2003, no. 12, 5 December 2003 (2003-12-05) & JP 2004 142261 A (KINO ORIMONO KK), 20 May 2004 (2004-05-20)

## Description

The present invention relates to methods for manufacturing fiber molded articles. More particularly, the present invention relates to methods for manufacturing fiber molded articles, e.g., fiber molded board, which comprise fibrous materials and binder materials.

Methods for manufacturing a fiber molded article such as a fiber molded board are known. In the known methods, fibrous materials such as resin-based fibrous materials or wood-based fibrous materials are bound via binder materials, i.e., thermoplastic resins or thermosetting resins. In the known art, the formed fiber molded article may have varying or uneven physical properties (e.g., unit strength, bending strength and resistance to debonding) that are caused by a nonhomogeneous distribution of the binder materials in the fibrous materials. Therefore, many approaches have been proposed for evenly feeding the binder materials into the fibrous materials.

One approach is taught, for example, by Japanese Patent Number 2718167. In this approach, the fibrous materials are impregnated with an aqueous suspension (dispersion liquid) of binder materials by spraying, thereby producing binder material-impregnated fibrous materials. After drying, the produced binder material-impregnated fibrous materials are assembled and heat treated so as to form a mat-shaped fiber product. Thereafter, the formed fiber product is molded by molding under heat and pressure, thereby manufacturing a fiber molded article. Another approach is taught, for example, by Japanese Laid-Open Patent Publication Number 2002-192507. In this approach, the fibrous materials (kenaf fibers) are previously assembled or pre-shaped so as to form a mat-shaped fiber product. The formed mat-shaped fiber product is dipped in liquefied phenol resins, thereby producing a phenol resin-impregnated mat-shaped fiber product. After drying, the produced phenol resin-impregnated fiber product is molded by molding under pressure, thereby manufacturing a fiber molded article. In addition, a different approach is taught, for example, by Japanese Laid-Open Patent Publication Number 2002-192507. In this approach, the fibrous materials are assembled and pre-shaped while blending with powder binder materials. The pre-shaped fibrous materials are then heat treated, thereby producing a resin-adhered fiber product. The resin-adhered fiber product thus produced is shaped by molding under heat and pressure, thereby manufacturing a fibre moulded article.

However, in the first to third approaches, two heat treating steps are required for manufacturing the fibre moulded article. As a result, the process for manufacturing the fibre moulded article is complicated and time consuming. Also, in the second approach it is difficult to control the amount of the impregnating resins because the fibre product is impregnated with the resins by dripping. Further, in the third approach the binder materials cannot be sufficiently or homogeneously combined with the fibrous materials because the binder materials are used in powdery form. In addition, the powdery binder materials may be easily removed from the fibrous materials (or localised within the fibrous materials), for example, when the pre-shaped fibrous materials are heat treated in order to adhere the binder materials to the fibrous materials.

Further, a fibre product that is impregnated with liquefied phenol resins or an aqueous binder material dispersion liquid can be directly moulded without drying, by moulding under heat and pressure. However, when such a fibre product is heated during moulding, the fibre product may be locally heated so that a suspension medium or a solvent of the resins is locally evaporated within the fibrous materials. As a result, the suspension medium or the solvent may flow toward the locally heated portion of the fibre product so as to move the impregnated resins within the fibrous materials. Thus, the resins may be unevenly dispersed in the fibrous materials.

US-A-4292105, GB-A-1453503, EP-A-1400328 and EP-A-2376051 describe other known methods for manufacturing fibre moulded articles.

It is, accordingly, an aim of the present invention to provide improved methods for manufacturing a fibre moulded article.

The present invention provides a method for manufacturing a fibre moulded article that comprises a fibrous material and a binder material, the method comprising:
producing a base product by applying a mat-shaped fibrous material with a binder material liquid that comprises the binder material dispersedly suspended and fluidized by a fluidizer;
drying the base product;
and moulding the dried base product under heat and pressure;
characterised in that the base product is dried under heat and pressure to ensure that the binder material is evenly disposed into the fibrous material without being squeezed out therefrom, in order to flow and evaporate the fluidizer contained in the base product before the base product is moulded, thereby dispersing the binder material within the base product;
in that the drying step is performed at a temperature between the boiling point of the fluidizer minus 20°C and the boiling point of the fluidizer plus 20°C and below the melting point of the binder material, and
in that the pressure in the drying step is produced by a pressing machine.

According to the present method, in the drying step, the fluidizer of the binder material liquid can be gently or slowly evaporated. Therefore, the fluidizer may effectively be prevented from flowing within the fibrous material of the base product. As a result, the binder material can be effectively prevented from migrating within the fibrous material of the base product.

Further, the binder material liquid can be smoothly penetrated into the fibrous material of the base product because the base product is effectively compressed. Therefore, the binder material can be evenly dispersed within the fibrous material.

Also, the fluidizer of the binder material liquid can be prevented from unevenly evaporating because the base product can be rapidly heated due to the applied pressure. Therefore, the fluidizer may effectively be prevented from flowing within the fibrous material of the base product. As a result, the binder material can be effectively stabilised within the fibrous material without being localised. Thus, according to the present method, it is possible to produce a fibre moulded article in which the binder material is homogeneously dispersed within the fibrous material. The fibre moulded article thus produced may have an excellent bending strength and a relatively good appearance.

Other aims, features and advantages of the present invention will be readily understood after reading the following detailed description together with the claims.

A representative embodiment of the present teachings will now be described in detail. According to the present teachings, a method will be provided for manufacturing a fibre moulded article. Further, the fibre moulded article that is manufactured utilising the present method includes various types of interior finishing members of vehicles and buildings, i.e., board-shaped members that can be moulded by various types of press forming including three-dimensional forming. More particularly, such a fibre moulded article includes, for example, but is not limited to, a door trim board, an instrument panel, and covering members for doors or furnishings.

In the present method, a fibrous material is previously assembled and shaped so as to make a mat-shaped fiber product. Conversely, a binder material that can bond or combine the fibrous material is mixed with a fluidizing medium or fluidizer that can dissolve or suspend the binder material, thereby formulating a binder material liquid. Consequently, the mat-shaped fiber product is then impregnated with the binder material liquid, thereby producing a binder material-impregnated mat-shaped base product (which will be simply referred to as a "base product") for manufacturing the fiber molded article. Further, an insert (e.g., a reinforcement member) can be embedded within the mat-shaped fiber product before it is impregnated with the binder material liquid so that the produced base product may contain such an insert therein, if necessary.

The base product thus produced is transferred to a drying step so as to be dried (i.e., so as to evaporate the fluidizer) by heating under pressure. Preferably, the base product is heated to a temperature between the boiling point (B) of the fluidizer minus 20°C and the boiling point (B) of the fluidizer plus 20°C (i.e., between B-20°C and B+20°C) and below the melting point (M) of the binder material (i.e., < M). In this drying step, the binder material liquid is penetrated into the fibrous material so that the binder material can be evenly dispersed into the fibrous material because the fibrous material of the base product is compressed due to the applied pressure. Therefore, when the base product is dried the binder material can be immobilized within the fibrous material in a condition such that the binder material is homogeneously dispersed therewithin. As a result, upon completion of the drying step the binder material can be stabilized or retained within the fibrous material without being localized.

The base product can be dried by means of various types of heating and pressing methods. For example, the base product can be dried by utilizing a pressing machine disposed within a heating furnace that can be heated to a desired temperature. Also, the base product can be dried by utilizing a pressing machine of which the pressing surfaces or die surfaces can be heated to a desired temperature. Further, the base product can be dried by pressing the base product to a desired thickness utilizing a pressing machine and by heating the pressed base product in a heating furnace.

As described above, the base product may preferably be heated to a temperature between the boiling point (B) of the fluidizer minus 20°C and the boiling point (B) of the fluidizer plus 20°C. If the base product is heated to a temperature below the boiling point of the fluidizer minus 20°C, the evaporation speed of the fluidizer may be extremely delayed. This may lead to prolongation of the drying time of the base product. To the contrary, if the base product is heated to a temperature above the boiling point of the fluidizer plus 20°C, the evaporation speed of the fluidizer may be extremely accelerated. As a result, the binder material can migrate along with the evaporating fluidizer. This may lead to an undesirable localization of the binder material within the fibrous material. Preferably, the base product is heated to a temperature between the boiling point (B) of the fluidizer and the boiling point (B) of the fluidizer plus 10°C (i.e., between B and B+10°C) in order to avoid the migration of the binder material caused by the rapid evaporation of the fluidizer. Typically, the base product is heated to a temperature of the boiling point of the fluidizer plus 10°C (i.e., B+10°C).

As will be easily understood, the base product is dried by appropriately controlling the pressure applied thereto. That is, the applying pressure is controlled such that the binder material liquid can sufficiently penetrate into the fibrous material without being squeezed out therefrom. Therefore, the amounts and strength of the pressure may preferably be controlled depending upon the types and conditions of the fibrous material and the amounts and flow properties of the fluidizer.

Generally, the base product is sufficiently dried until the fluidizer of the binder material liquid substantially evaporates so that flowability of the binder material liquid is substantially or completely faded away. Preferably, the base product is dried until the binder material liquid is substantially cured so as to not adhere to a carrier or other such members. Further, in a case that the fibrous material is natural fibers such as kenaf fibers that inherently contain water (i.e., water containing fibers), the base product is dried in consideration of such water if water or water compatible liquid is used as the fluidizer. For example, when the base product is composed of kenaf fibers and an aqueous binder material liquid, the base product is dried until the moisture content thereof is reduced to 10% by weight.

In the dried base product, the fibrous material is preferably densified so that the binder material is relatively evenly dispersed within the fibrous material and is reliably retained therewithin. Further, in this drying step the fluidizer is evaporated relatively slowly. Therefore, the binder material can be relatively evenly dispersed throughout the base product, in particular, in the direction of thickness.

The base product thus dried is then transferred to a forming step so as to be shaped or molded, thereby producing the fiber molded article. Typically, the dried base product is transferred to the forming step immediately after the drying step, i.e., before the heat applied to the base product during the drying step is removed therefrom. The reason is that if the dried base product is molded shortly after the drying step, it is possible to reduce the thermal energy and time required to mold the dried base product. Naturally, the dried base product can be tentatively stored before it is transferred to the forming step. Further, in the forming step, the base product can be molded with a covering member, thereby producing the fiber molded article covered with the covering member, if necessary. As will be appreciated, the produced fiber molded article may preferably be provided with attachment members (e.g., a retainer bracket) by fusion welding or adhering, if necessary.

In the forming step, the dried base product is molded by molding under heat and pressure. Typically, the base product is heated to a temperature (a fiber bonding temperature) that permit the binder material to bond or combine the fibrous material. When thermoplastic resins are used as the binder material, the fiber bonding temperature substantially corresponds to the melting point of the thermoplastic resins. Conversely, when thermosetting resins are used as the binder material, the fiber bonding temperature substantially corresponds to the setting temperature of the thermosetting resins.

The dried base product can be molded by means of various types of known molding methods. For example, when a thermoplastic resin is used as the binder material the dried base product is preheated within a heating furnace to a temperature above the melting point of the thermoplastic resin. Further, the heating furnace may preferably be controlled such that the base product is uniformly heated. Thereafter, the heated base product is molded by cold molding so as to produce the fiber molded article. Conversely, when a thermosetting resin is used as the binder material, the dried base product is molded by utilizing a molding machine of which the molding surfaces are heated to the a temperature above the setting temperature of the thermosetting resin. Further, the molding machine may preferably be controlled such that the base product is uniformly heated when molded. For example, both of the molding surfaces are heated such that the base product can be symmetrically heated along the direction of thickness.

As previously described, the binder material in the dried base product is relatively evenly dispersed within the fibrous material and is reliably retained therewithin. Therefore, even if the base product is compressed in the forming step the binder material can be prevented from migrating or localizing within the fibrous material. Consequently, the fibrous material can be relatively evenly bonded or combined by the binder material throughout the base product. Therefore, the fiber molded article produced from such a base product may have less "transparency (lack of hiding)" and "shrinkage." Further, as described above, the binder material in the base product is more evenly dispersed in the direction of thickness of the base product. Therefore, in a fiber molded article produced from such a base product the binder material is evenly dispersed throughout the article, in particular, in the direction of thickness of the article. In other words, the binder material is evenly present even in the core portion of the fiber molded article. Therefore, the fiber molded article may have an excellent resistance to debonding. In particular, when a combination of natural fibers and a biodegradable binder material is used in order to produce the base product, the fiber molded article may have an increased resistance to moisture and a good resistance to degradation due to humidity and heat. As a result, the fiber molded article may continuously keep a predetermined thickness and a desired strength for a long time.

Further details concerning the fibrous material, the binder material liquid (the binder material and the fluidizer) and the base product will now be described. The fibrous material used in the present embodiment may be various types of known fibers having a relatively long length as compared with the cross-sectional area thereof, e.g., plant-derived fibers, animal-derived fibers, chemical fibers (synthetic fibers), or other such fibers. Representative examples of the fibrous material may include bast fibers of bast plants (e.g., sisal and kenaf); fibers that are obtained by defibrating sugarcane bagasses or woods; cotton fibers; animal hairs; fibers of polyamide resins (nylon), acrylic resins, polyurethane resins and cellulosic resins (rayon). However, non-petrochemical fibers are appropriate for the fibrous material. Kenaf fibers (in particular, kenaf bast fibers) are suitable because they have a long fiber length. Also, kenaf fibers can be effectively and economically available because kenaf is an easily cultivable annual herb.

Further, the fibrous material may be a fiber blend of natural fibers (e.g., the plant-derived fibers and the animal-derived fibers described above) and synthetic fibers, which can melt and bond the natural fibers when heated in the forming step. The synthetic fibers that can be used in order to prepare such a fiber blend may preferably be thermoplastic resin fibers that are formed from thermoplastic resins. It is preferred that the thermoplastic resin fibers can be melted without damaging the natural fibers when they are heated to the fiber bonding temperature in the forming step described above. It is further preferred that the thermoplastic resin fibers not be melted when the fiber blend is heated in the drying step. If the thermoplastic resin fibers are melted or softened in the drying step, the dried base product may become sticky. Such a sticky base product may reduce workability.

Typically, the thermoplastic resin fibers of the fibrous material (the fiber blend) may preferably be formed from the same thermoplastic resins as the thermoplastic resins that can be used as a binder material. Examples of such thermoplastic resins may include polyolefins such as polyethylene and polypropylene; aliphatic polyester resins such as polylactic acid, polycaprolactone, and copolymers of hydroxycarboxylic acid with polylactic acid or polycaprolactone, in particular, hydroxy acid aliphatic polyester resins; polyesters such a PET (polyethylene terephthalate); acetyl cellulose (cellulose acetate) resins; and chemically modified starch resins. Preferably, the thermoplastic resins may be biosynthetically producible compounds such as polylactic acid and polycaprolactam; and plant-based compounds such as acetyl cellulose resins and chemically modified starch resins because these resins may have a reduced environmental load and save oil resources. More preferably, the thermoplastic resins may be polylactic acid because polylactic acid has excellent heat resistance and hardness and can reliably bond the natural fibers (the plant-derived fibers). Further, polyolefins, in particular, polypropylene may be useful in order to form the thermoplastic resin fibers because of their high bonding performance.

The thermoplastic resin fibers of the fiber blend may preferably be formed from thermoplastic resins similar to the thermoplastic resins of the binder material. Such thermoplastic resin fibers may cooperate with the binder material so as to reliably combine or bond the natural fibers. For example, when the binder material liquid is an aqueous suspension or an aqueous dispersion liquid that is formulated by mixing polylactic acid with water, the thermoplastic resin fibers may preferably be formed from polylactic acid.

The amount of the thermoplastic resin fibers may preferably be, but is not limited to, twenty (20) percent or less by weight of the total weight of the fibrous material (the natural fibers and the thermoplastic resin fibers) and the binder material. That is, the weight ratio of the natural fibers to the thermoplastic resin fibers to the binder material may preferably be 6-7:1-2:1-2, e.g., 7:1:2, 7:2:1 and 6:2:2. If the amount of the thermoplastic resin fibers is greater than 20 percent by weight of the total weight of the fibrous material and the binder material, the produced fiber molded article may have a reduced flexural strength. Also, if the amount of the thermoplastic resin fibers is greater than 20 percent by weight of the total weight of the fibrous material and the binder material, the weight of the produced fiber molded article may be increased.

The binder material of the binder material liquid may preferably be made from thermoplastic resins or thermosetting resins that can bond or combine the fibrous material. Examples of the thermoplastic resins may include polyolefins such as polyethylene and polypropylene; aliphatic polyester resins such as polylactic acid, polycaprolactone, and copolymers of hydroxycarboxylic acid with polylactic acid or polycaprolactone, in particular, hydroxy acid aliphatic polyester resins; polyesters such a PET; acetyl cellulose (cellulose acetate) resins; and chemically modified starch resins. Conversely, examples of the thermosetting resins may include polyurethane resins (resins formed from polyisocyanate and polyol), epoxy resins, phenolic resins and urea resins. Preferably, the thermoplastic resins may be biosynthetically producible compounds such as polylactic acid and polycaprolactam; and plant-based compounds such as acetyl cellulose resins and chemically modified starch resins, i.e., resins that are not derived from oil resources. More preferably, the thermoplastic resins may be polylactic acid because polylactic acid has excellent heat resistance and hardness and can reliably bond the natural fibers (the plant-derived fibers). For example, the base product that is produced from kenaf fibers and polylactic acid may not only save oil resources but also may be disposed without producing toxic substances that can deteriorate a working environment and consequently a natural environment.

The fluidizer of the binder material liquid may preferably be solvents that can liquefy the binder material (e.g., various types of organic solvents) or suspension media that can suspend the binder material (e.g., water). Examples of the fluidizer may include ethanol, acetone, water, and mixtures of water and ethanol. Water and water-based aqueous solutions are very suitable because they do not substantially produce toxic substances when evaporated in the drying step and the forming step. Also, the water-based solutions (e.g., a water-based ethanol solution) may effectively reduce the drying time in the drying step because such solutions can more easily evaporate than pure water.

Therefore, in view of the working environment and the natural environment, the suitable binder material liquid may be an aqueous thermoplastic resin dispersion liquid, e.g., an aqueous polylactic acid dispersion liquid (i.e., a suspension in which polylactic acid is dispersed in water or a water-based ethanol solution). Further, the binder material liquid (in particular, the binder material dispersion liquid or suspension) may contain surfactants, emulsifiers or other such additives, if necessary.

As described above, the fibrous material is previously assembled and shaped so as to make a mat-shaped fiber product. Typically, the mat-shaped fiber product may be a mat-shaped fiber assembly or a fortified mat-shaped fiber assembly. The mat-shaped fiber assembly is formed by simply assembling a desired amount (i.e., a desired weight per unit area) of the fibers or the fiber blend. Conversely, the fortified mat-shaped fiber assembly is formed by further treating the mat-shaped fiber assembly, e.g., by needle punching or thermo-compressing the same. The fortified mat-shaped fiber assembly may have excellent workability because of its ease of handling. In particular, when the fortified mat-shaped fiber assembly is formed by needle punching the mat-shaped fiber assembly that is made of a fiber blend of natural fibers (kenaf fibers) and thermoplastic resin fibers, the thermoplastic resin fibers can be reliably entangled with each other by needle punching because the thermoplastic resin fibers are more flexible than the natural fibers. Therefore, the fortified mat-shaped fiber assembly thus formed may have increased cutting characteristics and ease of handling characteristics. Also, because such a fortified mat-shaped fiber assembly can be obtained via a minimal needle punching operation, the natural fibers contained therein may not be damaged.

The mat-shaped fiber product (i.e., the mat-shaped fiber assembly or the fortified mat-shaped fiber assembly) may preferably be impregnated with the binder material liquid by means of various types of known methods, e.g., a spray application method, a roller application method and a dipping method. The spray application method and the roller application method are suitable because such methods can apply the binder material liquid to the mat-shaped fiber product such that the binder material liquid can be evenly dispersed in the fibrous material. Further, the binder material liquid can be applied to the mat-shaped fiber product in various directions. In addition, the binder material liquid can be pre-applied to the fibrous material before the fibrous material is assembled, if necessary.

The following examples show that the fiber molded article that is manufactured utilizing the present method has more excellent properties than the properties of the prior art fiber molded articles. Further, the following examples are illustrative and should not be construed as limitations of the invention.

### Example 1

In order to evaluate dispersion uniformity of the binder material liquid (the binder material) within the fibrous material of the fiber molded article, a plurality of samples of the fiber molded article (Samples A and B) were prepared utilizing the present method. Also, a control sample (Control A) was prepared utilizing a known method.

### Sample A:

Kenaf fibers (kenaf bast fibers) were assembled in an amount of 0.84 kg/m², thereby forming a mat-shaped fiber product. Polylactic acid (95 weight % or more L-form) was mixed with water, thereby formulating an aqueous dispersion liquid of polylactic acid, i.e., an aqueous polylactic acid dispersion liquid (30 weight % polylactic acid content). A desired amount of the aqueous dispersion liquid thus formulated was applied to the mat-shaped fiber product by spraying such that the amount of applied polylactic acid was about 30 weight % of the total weight of kenaf fibers and polylactic acid (i.e., such that the weight ratio of kenaf fibers to polylactic acid was 7:3), thereby producing a polylactic acid-impregnated mat-shaped base product. Thereafter, the base product was dried in a pressing machine of which the pressing dies were heated to 110°C, under a pressure of 15 kgf/cm² for three minutes. Subsequently, the dried base product was molded in a molding machine of which the molding dies were heated to 230°C, under a pressure of 24 kgf/cm² for 100 seconds, thereby producing a plate-shaped fiber molded article. At this time, the base product was heated to about 210°C. The produced fiber molded article had a weight per unit area of 1.2 kg/m².

### Sample B:

Similar to Sample A, kenaf fibers were assembled in an amount of 0.84 kg/m², thereby forming a mat-shaped fiber product. The formed mat-shaped fiber product was sliced or divided equally into two thinned parts having the same thickness. Thereafter, the aqueous polylactic acid dispersion liquid (30 weight % polylactic acid content) formulated as described above was applied to the upper surface of one part of the sliced fiber product. The amount of the aqueous dispersion liquid was substantially identical to the amount used in Sample A. One part thus treated was combined with the other part of the sliced fiber product such that the aqueous dispersion liquid, applied to the one part, was substantially sandwiched between the two parts, thereby producing a polylactic acid-impregnated mat-shaped base product. Thereafter, the base product was dried and molded under the same conditions as for Sample A, thereby producing a plate-shaped fiber molded article having weight per unit area of 1.2 kg/m².

### Control A:

Similar to Sample A, a polylactic acid-impregnated mat-shaped base product was produced. The base product thus produced was molded in a molding machine of which the molding dies were heated to 230°C, under a pressure of 24 kgf/cm² for 180 seconds, thereby producing a plate-shaped fiber molded article. At this time, the base product was heated to about 210°C. As will be recognized, the base product was not previously dried before it was molded.

Each of Samples A and B and Control A was sliced or divided equally into three thinned parts having the same thickness, i.e., an upper part, a middle part and a lower part. Thereafter, ten (10) mg specimens were taken from the upper part, the middle part and the lower part and placed into an aluminum cell. Conversely, ten (10) mg of pure (100%) polylactic acid (standard polylactic acid) that was treated by heating to 210°C was placed into an aluminum cell. Each of the cells that contained the specimens or the cell that contained pure polylactic acid and an additional empty cell were symmetrically disposed into a heating furnace. Thereafter, the heating furnace was heated to 210°C at a rate of temperature increase of 10°C/min so as to determine heat of fusion (J/g) of polylactic acid of each of the specimens and the standard polylactic acid at a temperature of 175°C. From the determined values of heat of fusion, a rate of resin content (%) in each specimen was calculated by the following equation: $Rate of Resin Content ( % ) = \frac{Heat of Fusion of Polylactic Acid of Specimen ( J / g )}{Heat of Fusion of Standard Polylactic Acid ( J / g )} \times 100$
Results are shown in Table 1. Further, the rate of resin content of each part is shown by an index number based on a minimum value (1.0) in these parts for comparison purposes.

**Table 1**

| | Rate of Resin Content (Index Number) | | |
|---|---|---|---|
| | Upper Part | Middle Part | Lower Part |
| Sample A | 1.1 | 1.0 | 1.0 |
| Sample B | 1.0 | 1.1 | 1.0 |
| Control A | 1.5 | 1.0 | 1.5 |

Table 1 demonstrates that each of Samples A and B has excellent dispersion uniformity of the binder material liquid (the binder material) within the fibrous material of the fiber molded article. That is, according to the fiber molded article prepared utilizing the present method, the binder material liquid (the binder material) may be substantially uniformly dispersed within the fibrous material along the thickness direction. On the contrary, in the Control A the binder material liquid (the binder material) is not uniformly dispersed within the fibrous material of the fiber molded article. That is, according to the fiber molded article prepared utilizing the conventional method, the binder material liquid (the binder material) is localized in the upper and lower parts.

### Example 2

In order to evaluate the bending strength and appearance of the fiber molded article, a plurality of samples of the fiber molded article (Samples 1-11) were prepared utilizing the present method. Also, a plurality of control samples (Controls 1-3) were prepared utilizing a known method.

### Sample 1:

A polylactic acid-impregnated mat-shaped base product was produced via the same process as in Sample A. Thereafter, similar to Sample A, the base product thus produced was dried. Subsequently, the dried base product was molded in the same molding machine and under the same conditions as for Sample A, thereby producing a plate-shaped fiber molded article. A part of the fiber molded article thus produced was then heated for three minutes in an oven at 235°C so as to be heated to 210°C. The heated fiber molded article thus produced was further molded (three-dimensionally molded) by cold molding, thereby producing a hat-shaped fiber molded article having a drawn portion 7 cm deep.

### Sample 2:

A polylactic acid-impregnated mat-shaped base product was produced via the same process as in Sample B. Thereafter, similar to Sample B, the base product was dried and molded, thereby producing a plate-shaped fiber molded article. A part of the fiber molded article thus produced was further molded via the same process as in Sample 1, thereby producing a hat-shaped fiber molded article.

### Sample 3:

Kenaf fibers (kenaf bast fibers) having a fiber length of 70 mm and fibers (6.6 dtex × 51 mm) made of polylactic acid (i.e., synthetic fibers) were assembled in an amount of 0.96 kg/m², thereby forming a mat-shaped fiber product. The weight ratio of kenaf fibers to the polylactic acid fibers was 7:1. Polylactic acid (95 weight % or more L-form) was mixed with water, thereby formulating an aqueous polylactic acid dispersion liquid (20 weight % polylactic acid content). A desired amount of the aqueous dispersion liquid thus formulated was applied to the mat-shaped fiber product by spraying such that the weight ratio of kenaf fibers to applied polylactic acid (the binder material) was 7:2, thereby producing a polylactic acid-impregnated mat-shaped base product. Thereafter, the base product thus produced was dried in a pressing machine of which the pressing dies were heated to 110°C, under a pressure of 15 kgf/cm² for three minutes. Subsequently, the dried base product was molded in a molding machine of which the molding dies were heated to 230°C, under a pressure of 24 kgf/cm² for 90 seconds, thereby producing a plate-shaped fiber molded article. At this time, the base product was heated to about 210°C. The produced fiber molded article had weight per unit area of 1.2 kg/m². A part of the fiber molded article thus produced was further molded via the same process as in Sample 1, thereby producing a hat-shaped fiber molded article.

### Sample 4:

Kenaf fibers (kenaf bast fibers) and fibers made of polylactic acid were assembled at an amount of 1.080 kg/m², thereby forming a mat-shaped fiber product. The weight ratio of kenaf fibers to the polylactic acid fibers was 7:2. Similar to Sample 3, an aqueous polylactic acid dispersion liquid (20 weight % polylactic acid content) was formulated. A desired amount of the aqueous dispersion liquid thus formulated was applied to the mat-shaped fiber product by spraying such that the weight ratio of kenaf fibers to polylactic acid (the binder material) was 7:1, thereby producing a polylactic acid-impregnated mat-shaped base product. Thereafter, the base product thus produced was treated via the same process as in Sample 3, thereby producing a plate-shaped fiber molded article. A part of the fiber molded article thus produced was further molded via the same process as in Sample 1, thereby producing a hat-shaped fiber molded article.

### Sample 5:

Kenaf fibers (kenaf bast fibers) and fibers made of polylactic acid were assembled in an amount of 0.84 kg/m², thereby forming a mat-shaped fiber product. The weight ratio of kenaf fibers to the polylactic acid fibers was 6:1. Similar to Sample 3, an aqueous polylactic acid dispersion liquid (20 weight % polylactic acid content) was formulated. A desired amount of the aqueous dispersion liquid thus formulated was applied to the mat-shaped fiber product by spraying such that the weight ratio of kenaf fibers to polylactic acid (the binder material) was 6:3, thereby producing a polylactic acid-impregnated mat-shaped base product. Thereafter, the base product thus produced was treated via the same process as in Sample 3, thereby producing a plate-shaped fiber molded article. A part of the fiber molded article thus produced was further molded via the same process as in Sample 1, thereby producing a hat-shaped fiber molded article.

### Sample 6:

Kenaf fibers (kenaf bast fibers) and fibers made of polylactic acid were assembled in an amount of 0.96 kg/m², thereby forming a mat-shaped fiber product. The weight ratio of kenaf fibers to the polylactic acid fibers was 6:2. Similar to Sample 3, an aqueous polylactic acid dispersion liquid (20 weight % polylactic acid content) was formulated. A desired amount of the aqueous dispersion liquid thus formulated was applied to the mat-shaped fiber product by spraying such that the weight ratio of kenaf fibers to polylactic acid (the binder material) was 6:2, thereby producing a polylactic acid-impregnated mat-shaped base product. Thereafter, the base product thus produced was treated via the same process as in Sample 3, thereby producing a plate-shaped fiber molded article. A part of the fiber molded article thus produced was further molded via the same process as in Sample 1, thereby producing a hat-shaped fiber molded article.

### Sample 7:

Kenaf fibers (kenaf bast fibers) and fibers made of polylactic acid were assembled at an amount of 1.08 kg/m², thereby forming a mat-shaped fiber product. The weight ratio of kenaf fibers to the polylactic acid fibers was 6:3. Similar to Sample 3, an aqueous polylactic acid dispersion liquid (20 weight % polylactic acid content) was formulated. A desired amount of the aqueous dispersion liquid thus formulated was applied to the mat-shaped fiber product by spraying such that the weight ratio of kenaf fibers to polylactic acid (the binder material) was 6:1, thereby producing a polylactic acid-impregnated mat-shaped base product. Thereafter, the base product thus produced was treated via the same process as in Sample 3, thereby producing a plate-shaped fiber molded article. A part of the fiber molded article thus produced was further molded via the same process as in Sample 1, thereby producing a hat-shaped fiber molded article.

### Sample 8:

This sample was produced similar to Sample 3 except that fibers made of polypropylene were used as the synthetic fibers.

### Sample 9:

This sample was produced similar to Sample 4 except that fibers made of polypropylene were used as the synthetic fibers.

### Sample 10:

This sample was produced similar to Sample 5 except that fibers made of polypropylene were used as the synthetic fibers.

### Sample 11:

This sample was produced similar to Sample 6 except that fibers made of polypropylene were used as the synthetic fibers.

### Control 1:

A polylactic acid-impregnated mat-shaped base product was produced via the same process as in Control A. Thereafter, the base product was molded in the same molding machine and under the same conditions as for Control A, thereby producing a plate-shaped fiber molded article. A part of the fiber molded article thus produced was further molded via the same process as in Sample 1, thereby producing a hat-shaped fiber molded article.

### Control 2:

Kenaf fibers (kenaf bast fibers) and fibers made of polylactic acid were assembled in an amount of 1.25 kg/m², thereby forming a mat-shaped fiber product. The weight ratio of kenaf fibers to the polylactic acid fibers was 7:3. The mat-shaped fiber product thus formed was directly molded in a molding machine of which the molding dies were heated to 230°C, under a pressure of 24 kgf/cm² for 60 seconds, thereby producing a plate-shaped fiber molded article. At this time, the fiber product was heated to about 210°C. The produced fiber molded article had weight per unit area of 1.2 kg/m². A part of the fiber molded article thus produced was further molded via the same process as in Sample 1, thereby producing a hat-shaped fiber molded article. As will be recognized, unlike Control 1, the fiber product was not impregnated with an aqueous dispersion liquid. That is, a dispersion liquid-impregnated mat-shaped base product was not produced before molding.

### Control 3:

This control was produced similar to Control 2 except that the weight ratio of kenaf fibers to the polylactic acid fibers was 6:4.

With regard to each of Samples 1-11 and Controls 1-3, the plate-shaped fiber molded article was partly cut away so as to form a 50 mm × 150 mm test piece. The test piece thus formed was used in order to determine the bending strength of the fiber molded article. The bending strength was determined by a three point bending method. That is, the bending strength was determined by pressing the central portion of a test piece that was supported at both longitudinal ends. From the determined values, the bending strength of the fiber molded article was evaluated based on the following reference levels:
A (Superior): not less than 30 Mpa
B (Inferior): less than 30 Mpa
Results are shown in Table 2.

In addition, with regard to each of Samples 1-11 and Controls 1-3, the hat-shaped fiber molded article was visually evaluated for the appearance, i.e., "tearing," "transparency (lack of hiding)" and "scuffing." The appearance of the fiber molded article was evaluated based on the following criteria:

### Tearing

A (Superior): no tearing
B (Ordinary): tearing without opening
C (Inferior): opening

### Transparency

A (Superior): no transparency
B (Ordinary): transparency without opening
C (Inferior): opening

### Scuffing

A (Superior): no scuffing
B (Ordinary): slight scuffing
C (Inferior): significant scuffing
Results are shown in Table 2.

**Table 2**

| | Bending Strength | Appearance | | |
|---|---|---|---|---|
| | | Tearing | Transparency | Scuffing |
| Sample 1 | A | A | C | C |
| Sample 2 | A | A | C | C |
| Sample 3 | A | A | A | B |
| Sample 4 | A | A | A | B |
| Sample 5 | A | A | A | A |
| Sample 6 | A | A | A | A |
| Sample 7 | B | A | A | A |
| Sample 8 | A | A | A | B |
| Sample 9 | A | A | A | B |
| Sample 10 | A | A | A | A |
| Sample 11 | A | A | A | A |
| Control 1 | A | C | C | C |
| Control 2 | B | B | C | B |
| Control 3 | B | A | A | A |

Table 2 demonstrates that the fiber molded article may have excellent bending strength when an aqueous dispersion liquid is applied to the kenaf fibers such that the amount of the binder material is not less than 20 weight % of the total weight of kenaf fibers, the synthetic fibers, and the binder material (Samples 1-6, 8-11 and Control 1). Also, Table 2 demonstrates that the fiber molded article may have inferior bending strength when synthetic fibers (the polylactic acid fibers) are added to the kenaf fibers such that the amount of the synthetic fibers is greater than 20 weight % of the total weight of kenaf fibers, the synthetic fibers, and the binder material (Sample 7 and Controls 2 and 3). This result indicates that it is preferable that the amount of the synthetic fibers is not greater than 20 weight % of the total weight of kenaf fibers, the synthetic fibers, and the binder material.

As will be apparent from Table 2, the fiber molded article in which synthetic fibers (the polylactic acid fibers) are not added to the kenaf fibers may generally produce "transparency" and "scuffing" (Samples 1 and 2 and Control 1). Also, the fibre moulded article in which the aqueous dispersion liquid is not used may generally produce an inferior appearance (Control 2). Further, the fibre moulded article in which the synthetic fibres (the polylactic acid fibres) are added to the kenaf fibres and in which the aqueous dispersion liquid is applied to the fibre blend may generally produce good results (Samples 3-11). In particular, the fibre moulded article in which the weight ratio of kenaf fibres to the synthetic fibres plus the binder material is 6:4 may produce good results (Samples 5-7, 10 and 11, and Control 3). This means that such a fibre moulded article can be suitably three-dimensionally moulded.

As a result, in order to produce a useful fibre moulded article having an increased bending strength and good appearance, it is preferable that synthetic fibres (e.g., the polylactic acid fibres) are added to the natural fibres (e.g., the kenaf fibres) so as to form the fibre blend. Further, it is preferable that the aqueous dispersion liquid of the binder material is applied to the fibres such that the weight ratio of the natural fibres to the synthetic fibres plus the binder material is 7:3-6:4.

This detailed description is merely intended to teach a person of skill in the art further details for practising preferred aspects of the present teachings and is not intended to limit the scope of the invention. Only the claims define the scope of the claimed invention. Therefore, combinations of features and steps disclosed in the foregoing detail description may not be necessary to practise the invention in the broadest sense, and are instead taught merely to particularly describe detailed representative examples of the invention.

## Claims

1. A method for manufacturing a fibre moulded article that comprises a fibrous material and a binder material, the method comprising:
producing a base product by applying a mat-shaped fibrous material with a binder material liquid that comprises the binder material dispersedly suspended and fluidized by a fluidizer;
drying the base product;
and moulding the dried base product under heat and pressure;
**characterised in that** the base product is dried under heat and pressure to ensure that the binder material is evenly disposed into the fibrous material without being squeezed out therefrom, in order to flow and evaporate the fluidizer contained in the base product before the base product is moulded, thereby dispersing the binder material within the base product;
**in that** the drying step is performed at a temperature between the boiling point of the fluidizer minus 20°C and the boiling point of the fluidizer plus 20°C and below the melting point of the binder material, and
**in that** the pressure in the drying step is produced by a pressing machine.

2. A method as claimed in claim 1, wherein the fluidizer comprises water, and wherein the drying step is performed at a temperature not less than 100°C and not greater than 110°C.

3. A method as claimed in claim 1 or claim 2, wherein the moulding step is performed at a temperature that permits the binder material to bond the fibrous material of the base product.

4. A method as claimed in any one of claims 1 to 3, wherein the fibrous material comprises natural fibres, and wherein the binder material liquid comprises an aqueous thermoplastic resin dispersion liquid.

5. A method as claimed in any one of claims 1 to 3, wherein the fibrous material comprises a fibre blend of natural fibres and thermoplastic resin fibres, and wherein the binder material liquid comprises an aqueous thermoplastic resin dispersion liquid.

6. A method as claimed in claim 4, wherein the aqueous thermoplastic resin dispersion liquid comprises an aqueous polylactic acid dispersion liquid.

7. A method as claimed in claim 5, wherein the thermoplastic resin fibres comprise polylactic acid fibres, and wherein the aqueous thermoplastic resin dispersion liquid comprises an aqueous polylactic acid dispersion liquid.

8. A method as claimed in claim 5, wherein the thermoplastic resin fibres comprises polypropylene fibres, and wherein the aqueous thermoplastic resin dispersion liquid comprises an aqueous polylactic acid dispersion liquid.

## Patentansprüche

1. Verfahren zur Herstellung eines Faserformkörpers, der ein Fasermaterial und ein Bindematerial aufweist, wobei das Verfahren Folgendes aufweist:
Erzeugen eines Grundprodukts durch ein Versetzen eines mattenförmigen Fasermaterials mit einer Bindemittelflüssigkeit, die das Bindematerial fein verteilt suspendiert aufweist und durch ein Verflüssigungsmittel verflüssigt ist;
Trocknen des Grundprodukts; und
Formen des getrockneten Grundprodukts unter Wärme und Druck;
**dadurch gekennzeichnet, dass**
das Grundprodukt unter Wärme und Druck getrocknet wird, um zu gewährleisten, dass das Bindematerial gleichmäßig in dem Fasermaterial verteilt ist, ohne aus diesem herausgedrückt zu werden, um das in dem Grundprodukt enthaltene Verflüssigungsmittel zu strömen und zu verflüchtigen bevor das Grundprodukt geformt wird, um **dadurch** das Bindematerial in dem Grundprodukt fein zu verteilen;
**dadurch**, dass der Trocknungsschritt bei einer Temperatur zwischen dem Siedepunkt des Verflüssigungsmittels minus 20°C und dem Siedepunkt des Verflüssigungsmittels plus 20°C und unterhalb des Schmelzpunkts des Bindematerials durchgeführt wird, und
**dadurch**, dass der Druck in dem Trocknungsschritt durch eine Pressmaschine erzeugt wird.

2. Verfahren nach Anspruch 1, wobei das Verflüssigungsmittel Wasser aufweist, und wobei der Trocknungsschritt bei einer Temperatur von nicht weniger als 100°C und nicht mehr als 110°C durchgeführt wird.

3. Verfahren nach Anspruch 1 oder 2, wobei der Formungsschritt bei einer Temperatur durchgeführt wird, die dem Bindematerial erlaubt, das Fasermaterial des Grundprodukts zu binden.

4. Verfahren nach einem der Ansprüche 1 bis 3, wobei das Fasermaterial Naturfasern aufweist, und wobei die Bindemittelflüssigkeit eine wässrige Thermoplastharz-Dispersionsflüssigkeit aufweist.

5. Verfahren nach einem der Ansprüche 1 bis 3, wobei das Fasermaterial eine Fasermischung von Naturfasern und Thermoplastharzfasern aufweist, und wobei die Bindemittelflüssigkeit eine wässrige Thermoplastharz-Dispersionsflüssigkeit aufweist.

6. Verfahren nach Anspruch 4, wobei die wässrige Thermoplastharz-Dispersionsflüssigkeit eine wässrige Polylactid-Dispersionsflüssigkeit aufweist.

7. Verfahren nach Anspruch 5, wobei die Thermoplastharzfasern Polylactidfasern aufweisen, und wobei die wässrige Thermoplastharz-Dispersionsflüssigkeit eine wässrige Polylactid-Dispersionsflüssigkeit aufweist.

8. Verfahren nach Anspruch 5, wobei die Thermoplastharzfasern Polypropylenfasern aufweisen und wobei die wässrige Thermoplastharz-Dispersionsflüssigkeit eine wässrige Polylactid-Dispersionsflüssigkeit aufweist.

## Revendications

1. Procédé pour fabriquer par moulage des articles contenant des fibres qui comprennent un matériau fibreux et un matériau de liaison, ou liant, le procédé comprenant:
- la production d'un produit de base par application d'ùn matériau fibreux sous forme de mat avec un matériau de liaison liquide, ou liant liquide, qui comprend le matériau de liaison, ou liant, sous la forme d'une dispersion en suspension et fluidisé par un fluidisant;
- le séchage du produit de base;
- et le moulage du produit de base séché sous l'action de la chaleur et de la pression;
**caractérisé**
* **en ce que** le produit de base est séché sous action de chaleur et de pression pour assurer que le matériau de liaison, ou liant, soit uniformément dispersé dans le matériau fibreux sans être chassé par excès de pression afin que le fluidisant contenu dans le produit de base s'écoule et s'évapore avant que le produit de base ne soit moulé, en dispersant ainsi le matériau de liaison, ou liant, à l'intérieur du produit de base;
* **en ce que** l'étape de séchage est effectuée à une température comprise entre le point d'ébullition, diminué de 20°C, du fluidisant et le point d'ébullition, augmenté de 20°C, du fluidisant, ladite température étant inférieure au point de fusion du matériau de liaison, ou liant, et
* **en ce que** la pression dans l'étape de séchage est produite par une machine de pressage.

2. Procédé selon la revendication 1, dans lequel le fluidisant comprend de l'eau, et dans lequel l'étape de séchage est effectuée à une température non inférieure à 100°C et non supérieure à 110°C.

3. Procédé selon la revendication 1 ou la revendication 2, dans lequel l'étape de moulage est effectuée à une température qui permet au matériau de liaison, ou liant, de lier le matériau fibreux du produit de base.

4. Procédé selon l'une quelconque des revendications 1 à 3, dans lequel le matériau fibreux comprend des fibres naturelles, et dans lequel le matériau de liaison liquide, ou liant liquide, comprend une dispersion aqueuse liquide de résine thermoplastique.

5. Procédé selon l'une quelconque des revendications 1 à 3, dans lequel le matériau fibreux comprend un mélange fibreux de fibres naturelles et de fibres de résine thermoplastique, et dans lequel le matériau de liaison liquide, ou liant liquide, comprend une dispersion aqueuse liquide de résine thermoplastique.

6. Procédé selon la revendication 4, dans lequel le liquide en dispersion aqueuse de résine thermoplastique comprend une dispersion aqueuse liquide d'acide polylactique.

7. Procédé selon la revendication 5, dans lequel les fibres de résine thermoplastique comprennent des fibres d'acide polylactique, et dans lequel le liquide en dispersion aqueuse de résine thermoplastique comprend une dispersion aqueuse liquide d'acide polylactique.

8. Procédé selon la revendication 5, dans lequel les fibres de résine thermoplastique comprennent des fibres de polypropylène, et dans lequel le liquide en dispersion aqueuse de résine thermoplastique comprend une dispersion aqueuse liquide d'acide polylactique.
